# EUROPEAN PATENT SPECIFICATION

(11) **EP 0 882 601 B1**
(45) Date of publication and mention of the grant of the patent: **28.02.2001**
(21) Application number: 98110033.2
(22) Date of filing: 02.06.1998
(51) Int. Cl.: B41M 5/34, B41M 5/38

(54) **Thermal transfer recording medium with wax release layer**
Thermische Übertragungsaufzeichnungsmaterial mit einer Abziehschicht aus Wachs
Matériau d'enregistrement pour le transfert par la chaleur avec une couche de décollage contenant une cire

(30) Priority: 03.06.1997 JP 14557497
(43) Date of publication of application: 09.12.1998
(73) Proprietor: FUJICOPIAN CO., LTD., Osaka-shi, Osaka-fu (JP); ALPS ELECTRIC CO., LTD., Ota-ku, Tokyo-to (JP)
(72) Inventor: Sogabe, Jun, Nishiyodogawa-ku, Osaka-shi, Osaka-fu (JP); Hoshino, Tetsuo, Nishiyodogawa-ku, Osaka-shi, Osaka-fu (JP); Asabe, Yoshiyuki, Otsukamachi, Ota-ku, Tokyo-to (JP); Arauchi, Susumu, Otsukamachi, Ota-ku, Tokyo-to (JP); Inoue, Yasutoshi, Otsukamachi, Ota-ku, Tokyo-to (JP); Ogiyama, Osamu, Otsukamachi, Ota-ku, Tokyo-to (JP)
(74) Representative: Bühling, Gerhard, Dipl.-Chem.

(56) References cited:
- EP-A- 0 510 661
- EP-A- 0 698 504
- US-A- 5 053 267

## Description

The present invention relates to a thermal transfer recording medium for use in thermal transfer recording devices such as thermal printers and facsimile terminal equipments. More particularly, the present invention relates to a thermal transfer recording medium for formation of a multi-color or full-color image by superimposing transfer of plural different color inks.

There has hitherto been conducted the formation of a multi-color or full-color image wherein plural different color inks are superimposingly transferred one on another on a receptor by means of a thermal transfer printer or the like to form a multi-color or full-color image involving a region developing a color by virtue of subtractive color mixture. As the thermal transfer recording medium for such a method there has been widely used one having the structure wherein a release layer comprising a wax as a main ingredient is interposed between a foundation and a color ink layer to improve the transferability.

When plural different color inks are superimposingly transferred to form a multi-color or full-color image on a receptor by use of the above-mentioned thermal transfer recording medium, the release layer comprising a wax as a main ingredient would exist on the top of first color ink dots formed on the receptor, thereby causing the problem wherein second color ink dots are not satisfactorily superimposed onto the first color ink dots due to the presence of the release layer on the first color ink dots.

EP-A-0 698 504 discloses a thermal transfer recording medium for color image formation including at least one region wherein different color ink dots are superimposed on each other to develop a color by virtue of subtractive color mixture. The recording medium comprises a foundation, a yellow heat-meltable ink layer, a magenta heat-meltable ink layer and a cyan heat-meltable ink layer disposed on the foundation in a side-by-side relation in a predetermined order and respective release layers each comprising a wax interposed between the foundation and the respective color ink layers. The melt viscosities at a predetermined temperature of the respective release layers corresponding to the respective color ink layers are stepwise decreased in the order in which the respective color ink layers are transferred. Such a thermal transfer recording medium exhibits good transferability and can give an increased dot-transfer ratio.

EP-A-0 510 661 discloses a sublimation transfer method and a heat-melt transfer medium. According to the sublimation transfer method, a heat-meltable ink layer containing a sublimation dye is melt-transferred to give a master having an image of the ink and the sublimation dye in the ink image is heat-transferred to form a dyed image on a substrate. According to the method, a heat-melt transfer medium is used, wherein a release layer comprising a wax-like substance as a major component is provided between a foundation and the ink layer, or an adhesive layer comprising a wax-like substance as a major component is provided on the ink layer or both the release layer and the adhesive layer are provided. The releasability of the ink layer from the foundation and the adhesiveness of the ink layers with each other are improved.

US-A-5,053,267 discloses a thermosensitive image transfer recording medium which comprises a support, a release layer formed on the support which comprises as the main component a thermofusable material and on which a transparent thermofusable ink layer is applied comprising a plurality of different color thermofusable ink sections formed side by side on the release layer. The melt viscosity of the thermofusable ink layer is larger than the melt viscosity of the release layer.

In view of the aforesaid problem of the prior art, it is an object of the present invention to provide a technique where in, in the case of forming a color image by use of a thermal transfer recording medium having the structure wherein a release layer comprising a wax as a main ingredient is interposed between a foundation and a color ink layer, second color ink dots are satisfactorily transferred onto first color ink dots.

This and other object of the present invention will become apparent from the description hereinafter.

The present invention provides a thermal transfer recording medium for forming a color image by superimposingly transferring plural different color inks, comprising a foundation and a color ink layer provided on the foundation, and a release layer comprising a wax interposed between the foundation and the color ink layer,
wherein the thickness d₁ of the release layer for a first color and the thickness d₂ of the release layer for a second color satisfy the relationship represented by formula (I):${\text{d}}_{\text{1}} {\text{< d}}_{\text{2}} {\text{< 2.0 d}}_{\text{1}}$

In an embodiment of the present invention, the thickness d₁ of the release layer for the first color is from 0.05 to 0.7 µm.

In another embodiment of the present invention, plural different color ink layers are disposed in a side-by-side relation on single foundation with respective release layers intervening therebetween.

In still another embodiment of the present invention, plural different color ink layers are disposed on separate foundations with respective release layers intervening therebetween.

Fig. 1 is a schematic sectional view showing a situation where a color image is formed by superimposing transfer using an example of the thermal transfer recording medium of the present invention on a thermal transfer printer.

Fig. 2 is a partial plan view showing a printing pattern of second color ink dots which is used in a printing test using the thermal transfer recording medium of the present invention.

The definition of the terms "first color" and "second color" used in the present invention is as follows: When two different color inks are superimposingly transferred one on the other, the one color which is transferred previous to the other color is "first color", and the other color which is transferred on the first color is "second color". For example, in the case of superimposingly transferring three different color inks of yellow (hereinafter referred to as "Y" in some cases), magenta (hereinafter referred to as "M" in some cases) and cyan (hereinafter referred to as "C" in some cases) in the order of Y, M and C, Y is a first color and M is a second color when the transfer of Y and M is taken in consideration, and M is a first color and C is a second color when the transfer of M and C is taken in consideration.

The definition of the terms "release layer for a first color" and "release layer for a second color" is as follows: The release layer which is interposed between a foundation and a color ink layer giving a first color is the release layer for the first color. The release layer which is interposed between a foundation and a color ink layer giving a second color is the release layer for the second color.

The thermal transfer recording medium of the present invention has the structure wherein a release layer comprising a wax as a main ingredient is interposed between a foundation and a color ink layer. The thermal transfer recording medium of the present invention includes two embodiments: One embodiment wherein plural different color ink layers are disposed in a side-by-side relation on single foundation with respective release layers intervening therebetween; and Another embodiment wherein plural different color ink layers are disposed on separate foundations with respective release layers intervening therebetween.

The thermal transfer recording medium of the present invention is characterized in that the thickness d₁ of the release layer for a first color and the thickness d₂ of the release layer for a second color satisfy the relationship represented by formula ( I ):${\text{d}}_{\text{1}} {\text{< d}}_{\text{2}} {\text{< 2.0 d}}_{\text{1}}$ and preferably the relationship represented by formula ( II ):${\text{1.1 d}}_{\text{1}} {\text{< d}}_{\text{2}} {\text{< 1.5 d}}_{\text{1}}$

By virtue of the feature that the thickness d₁ of the release layer for the first color and the thickness d₂ of the release layer for the second color satisfy the relationship represented by formula ( I ), preferably the relationship represented by formula ( II ), a desired effect that second color ink dots can be satisfactorily transferred onto first color ink dots can be exhibited.

The reason why the above-mentioned effect is exhibited will be explained by referring to the drawing.

Fig. 1 is a schematic sectional view showing the situation where a color image is formed by superimposing transfer using the thermal transfer recording medium of the present invention on a thermal transfer printer.

In Fig. 1, reference numeral 1 denotes a thermal transfer recording medium having the structure wherein a color ink layer 4 is provided on a foundation 2 with a release layer 3 intervening between the foundation 2 and the color ink layer 4. The recording medium 1 shown in Fig. 1 is adapted for the second color and the release layer 3 thereof has a thickness d₂. An ink image for the first color has been formed on a receptor (paper) B by using a recording medium for the first color (in Fig. 1, only one ink dot A is illustrated from the viewpoint of simple explanation). The ink dot A is composed of a color ink layer 4a fixed to the receptor B and a release layer 3a present on the color ink layer 4a.

The recording medium 1 for the second color is superposed on the receptor B having the ink dot A thereon. The combined recording medium 1/receptor B is heated from the side of foundation 2 with a thermal head (in Fig. 1, only one heating element T is illustrated).

The thickness d₂ of the release layer 3 for the second color is larger than the thickness d₁ of the release layer for the first color and, hence, larger than the thickness of the release layer 3a of the ink dot A for the first color. Generally, the thickness of the release layer of an ink dot thermally transferred is the same as or a few smaller than the original thickness of the release layer in the recording media After the combined recording medium 1/receptor B is heated with the heating element T in this state and the release layer 3 and the release layer 3a are melted, the release layer 3a of the ink dot A for the first color is cooled faster than the release layer 3 for the second color. Accordingly, when the recording medium 1 for the second color is peeled off from the receptor B, the cohesive force F₂ of the release layer 3 is smaller than the cohesive force F₁ of the release layer 3a and, as a result, the color ink layer 4 is peeled on the side of the release layer 3, so that an almost perfect ink dot for the second color is transferred onto the ink dot A for the first color. That is, the size of the ink dot for the second color is almost the same as the size of the ink dot A for the first color.

Thus, according to the present invention, ink dots for the second color are superimposingly transferred onto the ink dots in a predetermined region of a first color image, resulting in a desired subtractive color mixture to give a multi-color or full-color image with good color reproducibility.

When d₁ ≧ d₂, the ink dots for the second color are not satisfactorily transferred onto the ink dots for the first color, resulting in poor color reproducibility. When d₂ ≧ 2.0 d₁, it is difficult to transfer the ink dots for the second color with printing energy of the same level as that required for the transfer of the ink dots for the first color, resulting in complexity in setting the printing energy. In the present invention, from this point of view, it is preferable that d₁ and d₂ satisfy the relationship represented by formula ( II ):${\text{1.1 d}}_{\text{1}} {\text{< d}}_{\text{2}} {\text{< 1.5 d}}_{\text{1}}$

In the present invention, the thickness d₁ of the release layer for the first color is preferably from 0.05 to 0.7 µm. When the thickness of the release layer for the first color is smaller than the above range, the releasability of the release layer is prone to be insufficient. When the thickness of the release layer for the first color is larger than the above range, the release layer for the first color is not cooled faster than the release layer for the second color during the transfer of the ink dots for the second color onto the ink dots for the first color, and the cohesive failure is likely to occur within the release layer for the first color, resulting in unsatisfactory superimposing transfer of the ink dots for the second color.

When three colors, Y, M and C, are transferred in the order of Y, M and C, it is preferable that the thickness d₁ of the release layer for a first color is within the aforesaid range both in the case that a second color M is transferred onto a first color Y and in the case that a second color C is transferred onto a first color M.

With respect to other constitutents of the thermal transfer recording medium of the present invention, conventional ones can be adopted without any particular limitation so long as the release layers have respective thicknesses satisfying the aforesaid condition.

As the color ink layer there are usuallly used yellow, magenta and cyan ones. A black ink layer is optionally used. Usually, however, the black ink layer is not superimposed on other color ink layers. In that case, the release layer corresponding to the back ink layer does not need to satisfy the aforesaid condition.

These yellow, magenta and cyan ink layers and optionally a black ink layer may be disposed either on separate foundations or on single foundation.

According to an example of the thermal transfer recording medium wherein the respective color ink layers are disposed on single foundation, a yellow ink layer, a magenta ink layer and a cyan ink layer and optionally a black ink layer, each of which preferably has a given constant size, are repeatedly arranged in a side-by-side relation on single foundation in a recurring unit wherein the yellow, magenta and cyan ink layers and optionally the back ink layer are arranged in a predetermined order. The order of arrangement of these three or four ink layers in the recurring unit can be arbitrarily determined in consideration of the superimposing order of the respective color ink layers or the like. The respective release layers which are interposed between the foundation and the color ink layers in correspondence to the yellow, magenta and cyan ink layers and optionally the black ink layer are formed to have respective thicknesses satisfying the aforesaid condition in consideration of the transfer order of the respective color ink layers.

An example of the thermal transfer recording medium wherein the respective color ink layers are disposed on separate foundations comprises a combination of thremal transfer recording media comprising a first thermal transfer recording medium having a yellow ink layer on a first foundation, a second thermal transfer recording medium having a magenta ink layer on a second foundation and a third thermal transfer recording medium having a cyan ink layer on a third foundation, and optionally a fourth thermal transfer recording medium having a black ink layer on a fourth foundation. The respective release layers which are interposed between the respective foundations and color ink layers in correspondence to the yellow, magenta and cyan ink layers and optionally the black ink layer are formed to have respective thicknesses satisfying the aforesaid condition in consideration of the transfer order of the respective color ink layers.

Each of the release layers comprises a wax as a main ingredient thereof and may be incorporated with a thermoplastic resin, as required.

Examples of specific waxes include natural waxes such as lanolin, carnauba wax, candelilla wax, montan wax and ceresine wax; petroleum waxes such as paraffin wax and microcrystalline wax; synthetic waxes such as oxidized wax, synthetic ester wax, low molecular weight polyethylene wax, α-olefin-maleic anhydride copolymer wax, urethane wax, Fischer-Tropsch wax and synthetic petroleum wax. These waxes can be used either alone or in combination.

Examples of specific thermoplastic resins include ethylene-vinyl acetate copolymer, ethylene-alkyl (meth)acrylate copolymer, vinyl chloride-vinyl acetate copolymer, polyesters, polyamides, epoxy resins, petroleum resins and rosin resins. These resins can be used either alone or in combination.

The desired effect of the present invention can be effectively exhibited when the release layer for the first color and the release layer for the second color are the same or similar with each other in their compositions and/or physical properties. For example, with respect to the physical properties, it is preferable that the melting point and/or the melt viscosity of the release layer for the first color are the same as or similar to the melting point and/or the melt viscosity of the release layer for the second color within the melting point range of 60°C to 90°C and the melt viscosity range of 1 mPa·s to 1 Pa·s/100°C (1 to 1,000 cps/100°C).

Each of the color ink layers usable in the present invention is a heat-sensitive transferable color ink layer and comprises a coloring agent and a thermoplastic vehicle as main ingredients. The thermoplastic vehicle comprises a wax and/or a themoplastic resin. The desired effect of the present invention can be outstandingly exhibited when the color ink layer is one having relatively high cohesive force wherein the vehicle thereof comprises a thermoplastic resin as a main ingredient. From this point of view, each color ink layer preferably has a melt viscosity of 1 to 1·10³ Pa·s/160°C (10³ to 10⁶ cps/160°C).

Examples of specific waxes include natural waxes such as lanolin, carnauba wax, candelilla wax, montan wax and ceresine wax; petroleum waxes such as parafin wax and microcrystalline wax; synthetic waxes such as oxidized wax, synthetic ester wax, low molecular weight polyethylene wax, α -olefin-maleic anhydride copolymer wax, urethane wax, Fischer-Tropsch wax and synthetic petroleum wax. These waxes can be used either alone or in combination.

Examples of specific thermoplastic resins (inclusive of ealstomers) include ethylene copolymers such as ethylene-vinyl acetate copolymer, ethylene-vinyl butyrate copolymer, ethylene-(meth)acrylic acid copolymer, ethylene-alkyl (meth)acrylate copolymer wherein examples of the alkyl group are those having 1 to 16 carbon atoms, such as methyl, ethyl, propyl, butyl, hexyl, heptyl, octyl, 2-ethylhexyl, nonyl, dodecyl and hexadecyl, ethylene-acrylonitrile copolymer, ethylene-acrylamide copolymer, ethylene-N-methylolacrylamide copolymer and ethylene-styrene copolymer; poly(meth)acrylic acid esters such as polylauryl methacrylate and polyhexyl acrylate; vinyl chloride polymer and copolymers such as polyvinyl chloride, vinyl chloride-vinyl acetate copolymer and vinyl chloride-vinyl alcohol copolymer; polyesters, polyamides, epoxy resins, cellulose resins, natural rubber, styrene-butadine copolymer, isoprene polymer and chloroprene polymer; petroleum resins, rosin resins, terpene resins and cumarone-indene resins. These resins can be used either alone or in combination.

Coloring agents for yellow, magenta and cyan usable in the respective color ink layers are preferably transparent ones.

Examples of specific transparent coloring agents for yellow include organic pigments such as Naphthol Yellow S, Hansa Yellow 5G, Hansa Yellow 3G, Hansa Yellow G, Hansa Yellow GR, Hansa Yellow A, Hansa Yellow RN, Hansa Yellow R, Benzidine Yellow, Benzidine Yellow G, Benzidine Yellow GR, Permanent Yellow NCR and Quinoline Yellow Lake, and dyes such as Auramine. These coloring agents may be used either alone or in combination.

Examples of specific transparent coloring agents for magenta include organic pigments such as Permanent Red 4R, Brilliant Fast Scarlet, Brilliant Carmine BS, Permanent Carmine FB, Lithol Red, Permanent Red F5R, Brilliant Carmine 6B, Pigment Scarlet 3B, Rhodamine Lake B, Rhodamine Lake Y and Arizalin Lake, and dyes such as Rhodamine. These coloring agents may be used either alone or in combination.

Examples of specific transparent coloring agents for cyan include organic pigments such as Victoria Blue Lake, metal-free Phthalocyanine Blue, Phthalocyanine Blue and Fast Sky Blue, and dyes such as Victoria Blue. These coloring agents may be used either alone or in combination.

The term "transparent pigment" herein refers to a pigment which gives a tranparently colored ink when dispersed in a transparent vehicle.

Examples of coloring agents for black include pigments such as carbon black and Aniline Black, and dyes such as Nigrosine. These coloring agents may be used either alone or in combination.

The content of the coloring agent in each color ink layer is preferably from about 5 to about 60 % by weight. Each color ink layer may be incorporated with a dispersing agent, an antistatic agent or the like, as required. The thickness of each color ink layer is preferably from 0.5 to 2.0 µm.

As the foundation for the thermal transfer recording medium of the present invention, there can be used polyester films such as polyethylene terephthalate film, polyethylene naphthalate film and polyarylate film, polycarbonate film, polyamide film, aramid film, and other various plastic films commonly used for the foundation of ink ribbons of this type. Thin paper sheets of high density such as condenser paper can also be used. A conventionally known sticking-preventive layer may be provided on the back side (the side adapted to come into slide contact with a thermal head) of the foundation. Examples of the materials for the sticking-preventive layer include various heat-resistant resins such as silicone resins, fluorine-containing resins and nitrocellulose resins, and other resins modified with these heat-resistant resins, such as silicone-modified urethane resins and silicone-modified acrylic resins, and mixtures of the foregoing heat-resistant resins and lubricating agent. The thickness of the foundation is usually from 1 to 10 µm. From the viewpoint of reducing heat spreading to increase the resolution of images, the thickness of the foundation is preferably from 1 to 4.5 µm.

The formation of a color image with use of the thermal transfer recording medium of the present invention is preferably performed as follows: With use of a thermal transfer printer, the yellow ink layer (including the color ink layer and the corresponding release layer, hereinafter the same), the magenta ink layer and the cyan ink layer are selectively melt-transferred onto a receptor in a predetermined order according to respective separation color signals of an original color image, i.e. yellow signals, magenta signals and cyan signals to form yellow ink dots, magenta ink dots and cyan ink dots on the receptor in a predetermined order, yielding a yellow separation image, a magenta separation image and a cyan separation image superimposed on the receptor. The order of transfer of the yellow ink layer, the magenta ink layer and the cyan ink layer can be determined as desired. When a usual color image is formed, all the three color ink layers are selectively transferred according to three color signals to form three color separation images on the receptor. When only two color signals are present, the corresponding two of the three color ink layers are selectively transferred to form two color separation images of a yellow separation image, a magenta separation image and a cyan separation image. Thus there is obtained a multi-color or full-color image involving a color region wherein a color is developed by virtue of subtractive color mixture of superimposed two or three color inks.

Of course, the thermal transfer recording medium of the present invention can also be applied to the formation of a color image wherein superimposing transfer is performed by a heating means other than the thermal head, for example, irradiation with laser beam.

The present invention will be more fully described by way of Examples. It is to be understood that the present invention is not limited to the Examples.

### Examples 1 to 2 and Comparative Examples 1 to 3

A 2.5 µm-thick polyethylene terephthalate film provided on one side thereof with a 0.2 µm-thick sticking-preventive layer composed of a silicone-modified acrylic resin was used as a foundation. Onto the opposite side of the foundation with respect to the sticking-preventive layer was applied and dried a coating liquid for release layer with the following formula, thereby forming a release layer having a melting point of 75°C, a melt viscosity of 12 mPa·s/100°C (12 cps/100°C) and the thickness after being dried as shown in Table 2.

| Coating liquid for release layer | |
|---|---|
| Component | Part by weight |
| Paraffin wax | 8 |
| Toluene | 92 |

Onto the thus formed release layer was applied and dried a coating liquid for color ink layer (magenta or cyan) with the formula shown in Table 1 according to the combination shown in Table 2, thereby forming a 1.5 µm-thick color ink layer having a softening point of 65°C and a melt viscosity of 1.4·10² Pa·s/160°C (1.4 × 10⁵ cps/160°C).

With use of the thus obtained thermal transfer recording media, superimposing-printing was performed to determine the transfer ratio of the second color ink dot.

### <Evaluation method>

With use of the thermal transfer recording medium for cyan color (the first color), solid-printing was performed on a sheet of plain paper under the printing conditions mentioned below. Then, one-dot printing was performed in the pattern shown in Fig. 2 under the same printing conditions as above by using the thermal transfer recording medium for magenta color (the second color). In Fig. 2, reference numeral 10 denotes the solid-printed part for the first color, and reference numeral 11 denotes the second color ink dots.
Thermal transfer printer: PCPR 150V made by NEC corp.
Printing energy: 18 mJ/mm²
Printing speed: 100 characters per second
Size of heating element: 80 µm × 80 µm

With respect to the obtained printed matter, the transfer ratio of the second color ink dot defined by the following formula and the superimposing property was evaluated according to the following criterion. The results are shown in Table 2.$\text{Transfer ratio (%) =} \frac{{\text{Number of ink dots perfectly transferred /cm}}^{\text{2}}}{{\text{Total number of ink dots/cm}}^{\text{2}}} \text{× 100}$
A: Transfer ratio ≧ 90 %
B: 80 % ≦ Transfer ratio < 90 %
C: Transfer ratio < 80 %

**Table 1**

| Formula (part by weight) | Magenta | Cyan |
|---|---|---|
| Ethylene-vinyl acetate copolymer^{*1} | 60 | 60 |
| Petroleum resin | 10 | 10 |
| Carnauba wax | 10 | 10 |
| Billiant Carmine 6B | 20 | |
| Cupper Phthalocyanine Blue | | 20 |
| Toluene | 400 | 400 |

| | | |
|---|---|---|
| *1: Content of vinyl acetate: 28 % by weight, melt flow index: 150/190°C | | |

**Table 2**

| | Thickness of release layer (µm) | | Transfer ratio of second color ink dot (%) |
|---|---|---|---|
| | For cyan (first color) | For magenta (second color) | |
| Ex.1 | 0.5 | 0.7 | A |
| Ex.2 | 0.3 | 0.5 | A |
| Com.Ex.1 | 0.8 | 2.0 | C |
| Com.Ex.2 | 0.8 | 1.0 | B |
| Com.Ex.3 | 0.8 | 0.5 | C |

In addition to the materials and ingredients used in the Examples, other materials and ingredients can be used in Examples as set forth in the specification to obtain substantially the same results.

The thermal transfer recording medium of the present invention has the structure wherein a release layer comprising a wax as a main ingredient thereof is interposed between a foundation and a color ink layer. However, since the thickness d₁ of the release layer for the first color and the thickness d₂ of the release layer for the second color have the specific relationship, the second color ink dots can be satisfactorily transferred on the first color ink dots, resulting in a color image with good color reproducibility.

A thermal transfer recording medium for forming a color image by superimposingly transferring plural different color inks, comprising a foundation and a color ink layer provided on the foundation, and a release layer comprising a wax interposed between the foundation and the color ink layer,
wherein the thickness d₁ of the release layer for a first color and the thickness d₂ of the release layer for a second color satisfy the relationship represented by formula ( I ):${\text{d}}_{\text{1}} {\text{< d}}_{\text{2}} {\text{< 2.0 d}}_{\text{1}}$

## Claims

1. A thermal transfer recording medium (1) for forming a color image by superimposingly transferring plural different color inks, comprising a foundation (2) and a color ink layer (4) provided on the foundation, and a release layer (3) comprising a wax interposed between the foundation and the color ink layer,
wherein the thickness d₁ of the release layer (3a) for a first color (A) and the thickness d₂ of the release layer (3) for a second color satisfy the relationship represented by formula (I):${\text{d}}_{\text{1}} {\text{< d}}_{\text{2}} {\text{< 2.0 d}}_{\text{1}}$

2. The thermal transfer recording medium of Claim 1, wherein the thickness d₁ of the release layer for the first color is from 0.05 to 0.7 µm.

3. The thermal transfer recording medium of Claim 1, wherein plural different color ink layers are disposed in a side-by-side relation on single foundation with respective release layers intervening therebetween.

4. The thermal transfer recording medium of Claim 1, wherein plural different color ink layers are disposed on separate foundations with respective release layers intervening therebetween.

## Patentansprüche

1. Thermotransfer-Aufzeichnungsmedium (1) zur Erzeugung eines Farbbildes durch überlagertes Übertragen von mehreren unterschiedlichen Farbtinten, das folgendes umfasst: eine Unterschicht (2), eine auf der Unterschicht vorgesehene Farbtintenschicht (4) und eine Freisetzungsschicht (3), die ein zwischen der Unterschicht und der Farbtintenschicht eingefügtes Wachs umfasst,
wobei die Dicke d₁ der Freisetzungsschicht (3a) für eine erste Farbe (A) und die Dicke d₂ der Freisetzungsschicht (3) für eine zweite Farbe die durch die Formel (I) dargestellte Beziehung erfüllt:${\text{d}}_{\text{1}} {\text{< d}}_{\text{2}} {\text{< 2,0 d}}_{\text{1}}$

2. Thermotransfer-Aufzeichnungsmedium nach Anspruch 1, wobei die Dicke d₁ der Freisetzungsschicht für die erste Farbe zwischen 0,05 und 0,7 µm liegt.

3. Thermotransfer-Aufzeichnungsmedium nach Anspruch 1, wobei mehrere unterschiedliche Farbtintenschichten nebeneinander auf einer einzelnen Unterschicht mit dazwischenliegenden jeweiligen Freisetzungsschichten angeordnet sind.

4. Thermotransfer-Aufzeichnungsmedium nach Anspruch 1, wobei mehrere unterschiedliche Farbtintenschichten auf getrennten Unterschichten mit dazwischenliegenden jeweiligen Freisetzungsschichten angeordnet sind.

## Revendications

1. Milieu (1) d'enregistrement par transfert thermique pour former une image couleur en transférant avec superposition une pluralité d'encres de couleurs différentes, comprenant une base (2) et une couche d'encre de couleur (4) prévue sur la base, et une couche de décollement (3) comprenant une cire interposée entre la base et la couche d'encre de couleur, caractérisé en ce que l'épaisseur d₁ de la couche de décollement (3a) pour une première couleur (A) et l'épaisseur d₂ de la couche de décollement (3) pour une seconde couleur répondent à la relation représentée par la formule (I):${\text{d}}_{\text{1}} {\text{< d}}_{\text{2}} {\text{< 2,0 d}}_{\text{1}}$

2. Milieu d'enregistrement par transfert thermique selon la revendication 1, caractérisé en ce que l'épaisseur d₁ de la couche de décollement pour la première couleur est de 0,05 à 0,7 µm.

3. Milieu d'enregistrement par transfert thermique selon la revendication 1, caractérisé en ce qu'une pluralité de couches d'encres de couleurs différentes est disposée dans une relation côte à côte sur une base unique avec des couches de décollement respectives interposées entre elles.

4. Milieu d'enregistrement par transfert thermique selon la revendication 1, caractérisé en ce qu'une pluralité de couches d'encres de couleurs différentes est disposée sur des bases séparées avec des couches de décollement respectives interposées entre elles.
